

## UNITED STATES PATENT OFFICE

WILLIAM C. HAMPTON AND CHARLES N. GARBER, OF DAYTON, OHIO, ASSIGNORS TO THE CRAWFORD, McGREGOR AND CANBY COMPANY, OF DAYTON, OHIO, A CORPORATION OF OHIO

## METHOD OF COATING ARTICLES WITH PYROXYLIN OR THE LIKE

No Drawing.

Application filed June 18, 1930. Serial No. 460,786.

This invention relates to a method of coating articles of metal, wood, or other material with a surface covering of celluloid or pyroxylin applied in liquid form and subsequently 5 cured thereon to afford a continuous, one-piece, adherent envelope of substantially uniform thickness of quite considerable depth at a single operation and possessing a smooth and highly polished surface.

10 While reference is made in some prior patents to proposed applications of celluloid or pyroxylin as a coating material by dipping articles in a body of such materials in liquid form, such suggestions have been prophetic 15 only and the necessary teaching for successful working of pyroxylin materials in liquid form has been entirely lacking. Great difficulty is encountered in controlling the material subsequent to the dipping operation and 20 in effecting a curing of the coating material which will leave a finished surface undistorted and unblemished. Many unusual problems have been presented in effecting a 25 uniformly smooth polished surface deposit for which the hereinafter stated method affords a commercially practical solution.

The solvents employed in reducing pyroxylin and celluloid to liquid form are highly volatile, evaporating rapidly and permitting 30 the material to "set" quickly upon withdrawal from the dipping bath. Such rapid evaporation produces a refrigerating effect, causing precipitation of moisture from the surrounding atmosphere upon the coated surface. If 35 such moisture condensation trickles in streams upon the newly coated surface, it produces streaks and discoloration as well as distortion and a rough or matte surface. If such condensation stands in the form of dew, ice 40 crystals, or drops upon the freshly coated surface, it produces a rough and pitted surface effect. If the outer surface of the deposit is permitted to "set" too quickly, it forms an impenetrable film which prevents the 45 escape of the solvent from the inner strata and by un-uniform shrinkage of such outer surface film upon the inner material while yet in a soft condition, it induces wrinkling and produces a crinkled surface of intricate 50 design. If the freshly coated body is main-

tained at a moderate temperature sufficient to effect rapid evaporation of the solvent before such surface film can form, the solvent is quite likely to "boil" or vaporize within the deposit of coating material, thus forming 55 pimples and bubbles and causing the material to swell or "balloon" often assuming odd and grotesque shapes. From the experience of many such failures, the hereinafter method or process of successful treatment of articles 60 by dipping in liquid pyroxylin or celluloid has been evolved.

The object of the present invention is to provide a comparatively simple, economical, and commercially practical method for covering various articles of wood, metal and other materials, such as steering wheels for automobiles, door knobs, handles for cutlery, golf club heads and shafts, bathroom fixtures, toilet seats, and numerous other articles of 70 everyday commercial and household use with a covering of celluloid or pyroxylin having a uniformly smooth surface possessing a natural high polish or luster without the necessity of mechanical polishing or finishing operation, and of increased durability and capable of withstanding hard usage and wear, and which will provide a continuous one-piece covering without seams or joints, hermetically sealing the enclosed body against 75 entrance of moisture or attack by vapors or the like.

A further object of the invention is to provide an improved method or process of applying celluloid and pyroxylin in liquid form and controlling the resulting deposit to prevent "watering" from rapid evaporation, pitting or eggshell surface effect from dew or ice crystal deposits of moisture condensation, pimpling and bubble formation as result of "boiling" or vaporization of the contained solvent, and wrinkling or orange peel effect due to un-uniform shrinkage.

A further object of the invention is to provide a method and process by which various articles may be coated with celluloid or pyroxylin of various colors, giving to the articles pleasing and ornamental color effects.

A further object of the invention is to provide a method or process of encasing articles

within a covering of celluloid or pyroxylin of greater or less thickness, the extent of which may be controlled at will, and which may be deposited many times deeper than that of other finishing materials such as paints, lacquers, and varnishes, encasements having thickness of from twenty to sixty thousandths of an inch being ordinarily produced at a single dipping operation.

10 A further object of the invention is to provide a protective coating upon articles of wood, metal, and other material which will be tightly adherent, forming substantially a homogeneous body but which will at the same time possess sufficient flexibility to prevent cracking, chipping, crazing, and fracture.

15 A further object of the invention is to provide a coating or covering material which, when applied to articles possessing a degree of flexibility or resiliency such as shafts of golf clubs, canes, umbrella handles and the like, will yield in unison with the coated article.

20 With the above primary and other incidental objects in view, as will more fully appear in the specification, the invention consists of the steps and procedure, the apparatus and the method of operation or their equivalents as hereinafter described and set forth in the 25 claims.

25 In carrying out the present process, any suitable solvent for pyroxylin or for celluloid such as ether, alcohol, acetate, or the like, may be employed. However, acetone is the best known and preferable solvent for this 30 purpose. The process consists of three major operations, to wit, first the preparation and application of a rather thick, viscous solution of pyroxylin, second, the extraction of a 35 considerable portion of the solvent by chemical or other means as by plunging the coated article into a bath of liquid having a great affinity for the pyroxylin solvent and third, the evaporation of the remaining solvent by 40 governing such evaporation by temperature control and by preconditioning the air in which the curing of the material is effected.

45 Preparatory to the dipping or coating operation, the pyroxylin or celluloid, as the case may be, is thoroughly dissolved in a 50 suitable solvent until the material becomes a viscous, heavy liquid. This mixture of the material and the initial coating or dipping operation are best and preferably performed

55 in a room of normal temperature of approximately seventy degrees Fahrenheit. The viscous dipping solution takes approximately the same temperature or one somewhat lower due to the refrigerating effect of the evaporation of the solvent. The coating liquid is of 60 much thicker consistency than ordinary paint or lacquer, and therefore a quite heavy coating or deposit upon the article is obtainable.

65 After the article to be coated has been dipped into the liquid pyroxylin or celluloid

and the surplus material drained therefrom, the article being momentarily turned in various directions to insure distribution of the adhering material, it is immediately plunged or immersed in a bath of liquid which has an affinity for the pyroxylin solvent, and which is maintained at a comparatively low temperature, preferably a temperature below zero Fahrenheit.

70 The liquid coating material is very sensitive to temperature change, and when chilled becomes set into a semi-solid form in which the tendency to flow or change its shape is greatly retarded if not entirely overcome. Therefore the low temperature of the plunge bath has the effect of solidifying the coating material upon the article to such extent that it will maintain its shape and will overcome any tendency to flow or distort.

75 The liquid bath in which the coated article is immersed is preferably one having a great affinity for the pyroxylin solvent in which the solvent will readily mix or dissolve but in which the pyroxylin itself is insoluble. Such liquids as gasoline, benzine, benzol and the like, have been found quite practical in carrying out the present method. Such liquids while having a strong tendency to attract or dissolve the acetone or other solvents employed do not dissolve the cellulose, pyroxylin or celluloid to any appreciable extent, and, moreover, do not freeze but maintain substantially uniform fluidity at low temperature. Any liquid having these characteristics may be employed, that is, one having an affinity for the pyroxylin solvent and which is non-freezing, maintaining fluidity at low temperatures, and which will not be detrimental to the pyroxylin or other coating material. The liquids mentioned, i. e., gasoline, benzene and benzol may have a tendency to dissolve out the camphor contained in the celluloid or pyroxylin in the event that the work is left immersed too long in the bath. In the short time ordinarily required to set the coating material and to extract the solvent this effect upon the camphor content is negligible. However, under conditions where it may be found necessary to immerse the coated article for a longer period of time, the action of such bath liquid may be compensated for by adding a little excess camphor to the composition.

80 In lieu of maintaining the solvent extracting bath at an extremely low temperature, separate baths may be employed, one of which is a setting bath maintained at low temperature for solidifying the coating material and from which the coated article is transferred to a different bath at somewhat higher temperature by which the solvent is extracted but always maintained below the vaporization or boiling point of the solvent. The first or setting bath need not necessarily

possess the affinity for the solvent but may be merely a non-freezing solution which will be non-deleterious to the coating material and which is maintained at low temperature 5 sufficient to cause the quick setting of the material. Ordinarily the temperature of the initial bath whether of solvent extracting character or otherwise is maintained at from twenty to forty degrees below zero Fahrenheit. It is preferably, however, a bath of benzol, benzine, gasoline or the like in which the solvent is soluble and which has a great affinity for the solvent and so while solidifying the coating it also serves to extract some 10 of the solvent thus accelerating the setting or hardening of the material and preventing distortion. Extraction of solvent will, however, progress very slowly at such low temperature. At such temperature the bath has 15 little or no effect on the camphor content.

After being left in the initial bath sufficient time to become thoroughly chilled, which ordinarily requires from ten to fifteen minutes, the article is transferred to a second 20 bath of benzol, benzine, gasoline or other non-freezing material having great affinity for the solvent, which is maintained at a somewhat higher temperature of approximately zero Fahrenheit, by which the extraction 25 of the solvent is effected at a more rapid rate, and which results in further hardening and solidification of the coating material. When the greater portion of free solvent has 30 been removed and the action of the bath has diminished, the article may, if desired, be transferred to a third similar bath at a still higher temperature of approximately forty degrees Fahrenheit for the extraction of remaining solvent, the period varying according 35 to the size of the article and thickness of the coating. In practice, however, it is found that such third bath is but seldom necessary.

The difficulties ordinarily encountered due to the too rapid evaporation of the solvent 40 and deterioration and distortion of the coating material such as wrinkling, pimpling, and blushing or watering causing discoloration due to the refrigerating effect of the rapid evaporation, are overcome by the immersing of the coated article in this cold solvent-extracting bath. The low temperature of the bath changes the viscosity of the coating material so greatly that it becomes set almost immediately, and the absorption 45 or extraction of the solvent further increases the setting or hardening of the deposited pyroxylin material. However, this hardening or setting of the material is effected in the bath without the formation of an imper- 50 ous surface film which would tend to prevent the escape of any remaining solvent and result in wrinkling or pimpling. To the contrary upon removal from the bath, any remaining solvent may be freely evaporated 55 during the subsequent curing operation.

After removal from the liquid bath, the coated article is dried in a cold room from the air of which the moisture has been extracted to a point of low humidity so that the refrigerating effect of the evaporation of any 60 remaining solvent which tends to lower the temperature of the work will not cause moisture condensation. The drying or curing is preferably effected at a quite low temperature. A temperature of below zero Fahrenheit 65 is ordinarily employed, and a temperature as low as from twenty to fifty degrees Fahrenheit below zero has been found to be quite successful and practical. The work is maintained at low curing temperature until 70 substantially all of the solvent has been evaporated, thereby avoiding danger of wrinkling, pimpling or blistering due to the too rapid escape of solvent vapors or gases. After having been relieved of the solvent 75 vapors, the work is transferred to a room of somewhat higher temperature, preferably about thirty-two degrees Fahrenheit, where it is subjected to another period of drying. From this stage the work may be passed into 80 a room of normal atmospheric temperature and if a greater degree of hardening is required the work may be passed through successive stages of curing at higher tempera- 85 tures. 90

In the curing room advantage is taken of two physical conditions, i. e., the lowering of the temperature causes a lowering of the vapor tension, consequently the atmosphere 95 can contain less water vapor at the lower temperature than at a higher temperature, and advantage is also taken of the latent heat of evaporation. 100

Even though the temperature of the curing room be maintained quite low, the evaporation of the solvent nevertheless produces a refrigerating effect tending to lower the temperature of the coated article below that of the surrounding atmosphere and thereby induce on the surface coating condensation of moisture in the form of ice crystals. This effect, however, is counteracted by extracting the moisture from the air to a degree well below the saturation point before the air comes into contact with the coated article. 110 To this end the air entering the curing room is initially cooled to a quite low temperature. This room is maintained ordinarily at sub-zero Fahrenheit temperature and is preferably maintained at approximately forty degrees below zero Fahrenheit, although the degree of temperature may vary somewhat in accord with the particular material used and result desired. This chilling of the air causes the condensation of moisture therefrom in 115 the form of ice or frost, leaving the air comparatively dry, yet but little below the point of saturation at the resulting temperature. The temperature of the air is then slightly 120 raised to that of the curing room tempera- 125 130

ture. By raising the temperature of the curing air approximately five to ten degrees, not only is danger of moisture condensation by the refrigerating effect of the evaporating solvent removed, but the capability of the air to absorb the solvent vapors, which have a great affinity for moisture, is greatly increased. The slight warming of the air after it has been lowered to such temperature as to condense its entrained moisture, so increases its capacity to absorb and retain moisture that none of the small remaining amount of moisture in the air will be condensed upon the surface of the work, which, due to the evaporation effect of the solvent, is somewhat colder than the air circulating thereabout. The low temperature retards the evaporation of the solvent, allowing sufficient time for the solvent to escape from the deposited material without causing pimples or bubbles. The subjection of the coated article to such lowered temperature, also enables a heavier or deeper deposit to be retained upon the article than would otherwise be possible. Thus coverings or coatings of considerable thickness may be effected by a single dipping operation. To afford coverings of maximum thickness, the dipping and curing operations may be repeated several times.

The present material must not become confused with lacquers made from cellulose base, which are variously used and applied in liquid form. Such lacquers, although derived from the same base to which are added various gums and solvents, differ widely from the present material in character, being brittle and dry, lacking the tensile strength and durability, and can be practically applied only in thin coatings, whereas the present material can be applied to form a quite thick casing or shell about the article, which will be hard but tough and practically unbreakable.

Although the commercial material known as pyroxylin, pyroxyle, or pyroxylene, otherwise known specifically as celluloid, is the preferable material, the invention is not specifically limited to this material but includes other nitrocellulose derivatives or cellulose acetate having the characteristics of pyroxylin.

While the conditioning of the air in the curing room has been described as being cooled to a rather low degree to precipitate the moisture, and the temperature then raised to increase its vapor carrying capacity before it reaches the coated article, such air is not necessarily colder than the surface of the coated article with which the circulating air comes in contact. The evaporation of the solvent produces a refrigerating effect which tends to lower the temperature of the surface below that of the surrounding atmosphere even at the low temperature of the curing room.

The various temperatures herein mentioned are given for illustrative purposes only and with no intent to arbitrarily limit this invention to such stated temperatures nor relative temperature ranges. It is to be understood that the temperature and relative variations thereof may be varied within reasonable limits to meet different conditions of use, differences in the material composition and solvent employed, and results desired.

While only a few solvents for nitrocellulose material have been mentioned, and only a few liquids referred to for use as the intermediate setting bath and for extraction of the solvent, it will be understood that other solvents and other bath liquids having the necessary characteristics as hereinbefore described may be employed in lieu of those mentioned.

The pyroxylin material or the like may be cured in properly conditioned air alone without the use of the setting and solvent extracting bath. It may also be cured and the solvent extracted by the bath method alone to a point where the article may be exposed to air at atmospheric temperature without harmful effect. However, for practical commercial operation the hereinbefore described combined method of bath treatment followed by low temperature dry air treatment is preferred.

From the above description it will be apparent that there is thus provided a method of the character described possessing the particular features of advantage before enumerated as desirable, but which obviously is susceptible of modification in its steps, sequence, detail procedure and arrangement of apparatus without departing from the principle involved or sacrificing any of its advantages.

While in order to comply with the statute the invention has been described in language more or less specific as to structural features, it is to be understood that the invention is not limited to the specific details described, but that the means and method herein disclosed comprise the preferred form of several modes of putting the invention into effect, and the invention is, therefore, claimed in any of its forms or modifications within the legitimate and valid scope of the appended claims.

Having thus described our invention, we claim:

1. The herein described method of coating articles with pyroxylin or the like, consisting in dipping the portion of the article to be coated in a viscous solution of the coating material at approximately 70 degrees Fahrenheit, chilling the deposited coating to effect quick setting and preventing distortion of the deposit, extracting from the deposited material a portion of the coating material solvent and evaporating the remaining sol-

vent in an atmosphere of sub-zero temperature Fahrenheit and of low humidity characteristic.

2. The herein described method of coating articles with pyroxylin or the like, consisting in dipping the portion of the article to be coated in a viscous solution of the coating material, submerging the coated portion of the article in a cold bath having a temperature sufficiently low to cause the coating material to chill and set, and subsequently evaporating the solvent from the deposited material while maintaining the article at a low temperature.

3. The herein described method of coating articles with pyroxylin or the like, consisting in dipping the portion of the article to be coated in a viscous solution of the coating material, submerging the coated portion of the article in a bath of material having an affinity for the solvent and having a temperature of approximately 70° Fahrenheit less than that of the solution in which the article has been dipped whereby the material adhering to the article is congealed and a portion of the solvent is extracted from the deposit of coating material and subsequently evaporating from the deposited material the remaining solvent.

4. The herein described method of coating articles with nitrocellulose material consisting in dipping the article into a solution of the coating material, dipping the coated article into a bath of material having an affinity for the solvent and maintained at a temperature sufficiently low to effect a chilling and setting of the coating material and subsequently curing the coated article in a sub-zero Fahrenheit temperature.

5. The herein described method of coating articles with pyroxylin or the like consisting in dissolving the material in a solvent to form a viscous liquid, dipping the article to be coated in the viscous liquid at approximately normal atmospheric temperature, dipping the coated article in a bath maintained at a materially lower temperature to set the material, and subsequently evaporating the remaining solvent in an atmosphere from which moisture has been extracted at a sub-zero Fahrenheit temperature.

6. A method of coating articles with pyroxylin or the like consisting in dissolving the coating material to a viscous liquid, dipping the portion of the article to be coated into such liquid, draining therefrom the surplus material, submerging the coated portion of the article in a hardening and setting bath having a temperature materially lower than that of the viscous liquid in which the article has been dipped whereby the coating material is congealed thereon, and subsequently evaporating from the coating material any remaining solvent.

7. A method of coating articles with py-

roxylin or the like consisting in dissolving the coating material to a viscous liquid, dipping the portion of the article to be coated into such liquid, draining therefrom the surplus material, submerging the coated portion of the article in a body of material having an affinity for the coating material solvent maintained at the temperature materially lower than that of the liquid in which the article has been dipped by which the material is congealed and by which a considerable portion of the solvent is extracted prior to curing, and subsequently curing the coating material at low temperature.

8. A method of coating articles with pyroxylin or the like consisting in dissolving the coating material to a viscous liquid, dipping the portion of the article to be coated into such liquid, draining therefrom the surplus material, initially congealing the coating material to prevent displacement, extracting from the deposited coating material a considerable portion of the solvent and subsequently evaporating the remainder of the solvent while maintaining the coated article at a temperature materially lower than that of the liquid in which the article has been dipped.

9. A method of coating articles with pyroxylin or the like consisting in dissolving the coating material to a viscous liquid, dipping the portion of the article to be coated into such liquid, draining therefrom the surplus material, temporarily submerging the coated article in a bath of petroleum distillate to effect extraction of the solvent and evaporating remaining solvent from the coated article in a sub-zero temperature.

10. A method of coating articles with pyroxylin or the like consisting in dissolving the coating material to a viscous liquid, dipping the portion of the article to be coated into such liquid, draining therefrom the surplus material, submerging the coated article in a bath of petroleum distillate maintained at low temperature to set the deposited coating material by simultaneously chilling the material and extracting the solvent, and subsequently evaporating the remaining solvent at a sub-zero Fahrenheit temperature.

11. A method of coating articles with pyroxylin or the like consisting in dissolving the coating material to a viscous liquid, dipping the portion of the article to be coated into such liquid, draining therefrom the surplus material, chilling the deposited material to set and harden the same, extracting a portion of the solvent, evaporating the remaining solvent at a sub-zero Fahrenheit temperature and gradually raising the temperature of the coated article through successive stages.

In testimony whereof, we have hereunto set our hands this 26 day of May A. D. 1930.

WILLIAM C. HAMPTON.  
CHARLES N. GARBER.